

## UNITED STATES PATENT OFFICE

2,020,496

## PROCESS OF DYEING

Paul Bolen, Atlanta, Ga., assignor, by mesme assignments, to American Lecithin Company, Cleveland, Ohio, a corporation of Ohio

No Drawing. Application May 16, 1932,  
Serial No. 611,753

15 Claims. (Cl. 8—5)

The present invention relates to improvements in the art of sulphur, carbazole and vat dyeing processes. As is well known to those skilled in the art, the foregoing dyestuffs are insoluble in water in their oxidized state, but are soluble in their leuco form. In order to render these dyestuffs soluble in water, they are reduced in a strongly alkaline solution. Thus, the sulphur and carbazole dyestuffs are ordinarily obtained in solution by reducing them with  $\text{Na}_2\text{S}$  in a concentrated solution of soda ash, while the vat dyes are rendered soluble by reducing the same with sodium hydrosulphite in a concentrated solution of  $\text{NaOH}$ . Some of the carbazole dyestuffs are not reducible and rendered soluble by reduction with sodium sulphide in the presence of  $\text{Na}_2\text{CO}_3$ , but must be solubilized by reduction with  $\text{NaOH}$  and sodium hydrosulphite. Broadly speaking, sulphur and carbazole dyes are vat dyestuffs, because they are insoluble in water, but may be solubilized by alkaline reduction. However, the practical dyer considers sulphur dyes to be those water insoluble dyes which are solubilized by reduction with sodium sulphide in a hot concentrated solution of sodium carbonate, and which dye cotton, usually at the boil. Vat dyes on the other hand, are considered by the practical dyer, to be those dyestuffs which are solubilized by reduction with sodium hydrosulphite in a rather concentrated solution of sodium hydroxide. And intermediate between these two extremes, lie the carbazole dyes, some of which may be solubilized in the same manner as sulphur dyes, and others requiring the more energetic reduction provided for in the case of what the practical dyer considers a vat dye.

One of the major difficulties in the application of sulphur, carbazole or vat dyestuffs to the fibrous material is premature oxidation. This difficulty is particularly troublesome in the vat dyeing of piece goods in a dyeing jigger, because when cotton piece goods are dyed in a jigger with a vat dye, the selvedges of the goods which are more accessible to the atmosphere than the central portion of the piece goods, are oxidized by the oxygen of the air with the result that the piece is "side-shaded", or in other words, the sides of the piece are deeper or fuller in shade than the central portion. Of course such a result is highly unsatisfactory. The mode of procedure in jigger dyeing is such that it is very difficult to prevent this "side-shading", since the operation is slow and any given portion of the cloth is immersed in the dye bath for a comparatively short period of time. For example,

let us assume that 1,000 yards of cotton about 36 inches wide and weighing about  $\frac{1}{2}$  pound per yard is to be dyed a khaki shade with indanthrene dyestuffs. The depth of the shade together with the weight of the piece goods will require that the dye liquor contain several pounds of dyestuffs. In order to acquire the depth of shade necessary the dyeing operation proper (exclusive of oxidation and washing steps) will require about eight "ends" or eight passages through the dye liquor, each "end" consuming about ten minutes. The dyeing operation will consume, therefore, about one hour and twenty minutes, and it is very difficult to keep the dyestuff in a reduced state for this period of time. It will be found that edges of the roll of cloth being dyed will have become at least partially oxidized. In obtaining a khaki shade with indanthrene dyestuffs, indanthrene brown, olive and yellow are employed and the vat is a wine color. Now as the dyeing operation proceeds, it will be observed that the edges of the roll will not be wine colored, but will be greenish yellow in color, indicating oxidation. To offset as much as possible the premature oxidation, sodium hydrosulphite is added during the dyeing operation, usually at the end of a half hour.

Also, the addition of other types of reducing agents such as zinc-formaldehyde-sulfoxylate and the like has been proposed. The addition of acetone to the dye liquor tends to stabilize sodium hydrosulphite solutions.

In order to prevent premature oxidation I employ a suitable amount of lecithin, such as might be obtained from soya beans, dispersed in aqueous solution (for example the dye solution or dye liquors) by the aid of suitable emulsifiers or other colloidal media, such as the potassium and/or sodium salt of naphthenic acid, sodium and/or potassium salts of the fatty acids; or such as suitable solvents as phenyl carbinol, butyl cellosolve and the like, or mixtures of any of these materials.

This mixture may be added to the dyestuff or to the paste before reduction or to the reduced solution or to the dye bath proper, or at any other convenient point.

The correct amount to be used would depend on the type of dyeing apparatus and other conditions. For instance, the open type machines (jiggers and the like) would require more than the closed type (closed kettles and the like), since the dye liquor comes in contact with more air, hence oxidation takes place to a greater extent.

It varies between 0.5% and 3.0% of lecithin on the weight of material being treated.

In order to describe the invention more completely, the following specific examples are given 5 by way of illustration.

*Example I*

In preparing a dye bath containing Ciba brown R Colour Index No. 1187 concentrated powder, I

- 10 first prepare a paste containing 2,000 c. c. of NaOH solution of 66° Twaddell and 1,000 grams of the above dyestuff. When a uniform paste has been produced I introduce the same into 80 liters of water, maintained at a temperature of 15 70° C., continuously stirring the mixture. 1200 grams of sodium hydrosulphite are then slowly added and stirring is continued until reduction is complete, as indicated by the appearance of the brownish yellow colored vat. I then add 200 grams of soya bean lecithin containing 60% lecithin. The solution is cooled to 20/30° C., and diluted with twenty volumes of water to produce the final bath. The dyeing operation is carried out at 20/30° C.

25 *Example II*

In preparing a dye bath containing Cibanone red 4B Colour Index Supplement page 35, concentrated powder, I prepare a paste, containing 5,000 c. c. of NaOH solution of 66° Twaddell and 30 1,000 grams of the dyestuff. This paste is diluted with 100 liters of water maintained at a temperature between 40 and 50° C. 7500 grams of sodium hydrosulphite are then added and the mixture is stirred until reduction is complete, as indicated by the appearance of the blue red colored vat. This reduced liquor may be diluted with twenty volumes of water. I then add 150 grams of soya bean lecithin.

40 *Example III*

A dye bath containing Cibanone black B may be prepared in the manner described in the preceding examples, using 1,000 grams of the dyestuff, 5,000 c. c. of 66° Twaddell NaOH solution, 45 150 liters of water and 2,000 grams of hydrosulphite, reduction taking place at 60° C. I may add 175 grams of lecithin to the paste or I may add it to the reduced vat, either before or after final dilution. The dye is applied to the fiber at a temperature lying between 60 and 80° C.

It will be understood that in the above examples the amount of dyestuff used per given weight of cotton or other fibrous material will 55 depend on the shade desired. These examples are very broad types and show a wide range of temperatures, proportions and so forth.

In carrying out the invention in connection with the sulphur dyestuff I may proceed as follows.

60 *Example IV*

I first prepare a smooth paste containing 5,000 grams of Pyrogene deep black B Colour Index No. 991, in 20,000 grams of warm water. I then add 5,000 grams of crude sodium sulphide and 65 2,000 grams of soda ash. The mixture is thoroughly stirred while heating to 100° C. I then add 500 grams of soya bean lecithin before final dilution of the dye liquor.

70 *Example V*

I first prepare a smooth paste containing 5,000 grams Pyrogene brown 4R extra concentrated Colour Index No. 51, 20,000 grams of warm wa-

75 ter, 10,000 grams of crude sodium sulphide, 2,000 grams soda ash and 500 grams of lecithin obtained from skim milk. The paste is diluted with 10,000 grams of water and is reduced by heating to 50 to 70° C., while stirring. The solution is diluted to give the desired depth of shade.

In preparing a dye bath containing a carbazole dyestuff, I proceed as follows.

*Example VI*

Ciba blue 2 RH page 34 of Supplement to Colour Index, 1 pound color, 10 gallons water, 2 1/2 pounds NaOH 76%, 1 1/4 pounds hydro, 2 ounces lecithin, reduce 180° F. dye at 140° F., reddish yellow reduction.

15 *Example VII*

Ciba yellow G Colour Index No. 1196, 1 pound color, 10 gallons water, 2 1/4 pounds NaOH, 1 1/4 pounds hydro, 2 1/2 ounces lecithin, reduce at 20 150° F. dye at 120° F., reddish violet reduction.

In the foregoing examples, it will be observed that only one dyestuff has been used in preparing the bath. As a matter of fact a mixture of three or four dyestuffs are used in actual practice in order to obtain a given shade. This fact is well known to the practical dyer and he can readily observe from the proportions of dyestuff and lecithin set forth above, the amount of lecithin that should be used with a given weight of dyestuff, that is the total weight of the mixture of dyestuffs where such mixture is used. Also vat dyes usually are sold in the form of a 20% paste, by the manufacturer, and since the above proportions are based on the weight of dry powder, the dyer must take this fact into consideration.

Certain types of dyestuff, for instance Ciba yellow G, extra concentrated Colour Index No. 1196, cannot be run as self shades except for tinting on the continuous dyeing machines (piece goods or warps). In fact, practically all vat colors are limited to a medium shade on this particular machine. The reasons for this are that the fact the dyestuff in the high concentration necessary, would be prematurely oxidized. That, of course, causes inferior dyeing results, such as specks of precipitated dyestuff, excess foam marks, unevenness of shade, and the fastness is not in keeping with that expected from this class of dyestuffs. In the present practice, Cibanone blue G Colour Index No. 1195, is limited to concentrations of 5 ounces of dyestuff per gallon; Cibanone brown GR paste Colour Index No. 1173 is limited to 16 ounces per gallon of liquor; Cibanone blue 3G double paste is limited to 3 ounces per gallon. With the aid of lecithin this concentration can be increased to a point where the operation is profitable, considering the increase in concentration of dyestuff which is used, and the increase in the amount of color that a given quantity of dyestuff will produce. At the same time, the reduction can be maintained over a sufficient period of time to allow the running of adequate yardage to make the operation profitable. For instance, Cibanone blue G double paste Colour Index No. 1115, 5 ounces per gallon will run not over eighty minutes after reduction, whereas with the aid of lecithin it will run approximately double that time, or 160 minutes.

70 While I do not wish to limit myself to any particular theory, I am of the opinion that lecithin prevents premature oxidation by the mechanism of selective absorption of oxygen and also that the lecithin forms a protective shield, which pro-

tects the reduced dyestuff from the oxygen of the air.

As indicated previously, the lecithin may be added at any convenient stage of the dyeing process, that is it may be added to the original paste or to the diluted mixture of dyestuff and reducer, either before or after reduction.

Having disclosed the nature of my invention, what I claim is:

- 10 1. A process for dyeing fibrous material with a dyestuff which is soluble only in an alkaline medium, and by virtue of an alkaline reducing agent which comprises preparing a reduced alkaline solution of the dyestuff containing lecithin, and immersing the said fibrous material therein.
  - 15 2. A process for dyeing fibrous material with a water insoluble dyestuff which may be dissolved in an alkaline reducing medium, which comprises adding a small quantity of lecithin to the dyestuff, adding the dyestuff to an alkaline reducing medium while stirring to facilitate reduction and immersing the said fibrous material therein.
  - 20 3. A process for dyeing fibrous material with a vat dyestuff which comprises preparing a reduced alkaline solution of the said dyestuff containing a small quantity of lecithin and immersing the said fibrous material therein.
  - 25 4. A process for dyeing fibrous material with a vat dyestuff which comprises reducing the said vat dyestuff in an alkaline reducing medium, adding a small quantity of lecithin and immersing the said fibrous material therein.
  - 30 5. A process for dyeing fibrous material with a sulphur dyestuff which comprises preparing a reduced alkaline solution of the said dyestuff containing a small quantity of lecithin and immersing the said fibrous material therein.
  - 35 6. A process for dyeing fibrous material with a sulphur dyestuff which comprises reducing the said sulphur dyestuff in an alkaline reducing
  - 40
- medium, adding a small quantity of lecithin and immersing the said fibrous material therein.
7. A process for dyeing fibrous material with a carbazole dyestuff which comprises reducing the said carbazole dyestuff in an alkaline reducing medium, adding a small quantity of lecithin and immersing the said fibrous material therein.
8. A process for dyeing fibrous material with a carbazole dyestuff which comprises preparing a reduced alkaline solution of the said dyestuff containing a small quantity of lecithin and immersing the said fibrous material therein.
9. As a new composition of matter, a vat dye bath containing lecithin.
10. A process for dyeing fibrous material with a water insoluble dyestuff which may be dissolved in an alkaline medium and by virtue of an alkaline reducing agent, which comprises preparing a reduced alkaline solution of the dyestuff containing a small amount of lecithin and immersing the said fibrous material therein.
11. A process for dyeing fibrous material with a water insoluble dyestuff which may be dissolved in an alkaline medium and by virtue of an alkaline reducing agent, which comprises preparing a reduced alkaline solution of the dyestuff containing a small amount of lecithin, at least 2.5% by weight of the dyestuff, and immersing the said fibrous material therein.
12. As a new composition of matter, a sulphur dye bath containing lecithin.
13. As a new composition of matter, a carbazole dye bath containing lecithin.
14. A new composition of matter for addition to an alkaline reducing bath comprising a vat dye paste containing lecithin.
15. A new composition of matter for addition to an alkaline reducing bath, a dyestuff of the group consisting of vat, sulphur and carbazole dyestuffs in powder form, containing lecithin.

PAUL BOLEN.